

Patented Apr. 3, 1928.

1,664,742

# UNITED STATES PATENT OFFICE.

FERDINAND WYCLIFFE ELLINGTON, OF JAMAICA, NEW YORK.

## METHOD OF FINISHING LEATHER.

No Drawing.

Application filed August 27, 1926. Serial No. 132,038.

This invention relates to the method of gilding leather such as employed in making shoes, slippers, pocket books and other articles of manufacture using pure leather or 5 leather compositions.

One of the objects of my invention is to provide means for and the method of gilding leather in such a manner as to bring out in relief as far as possible the grain 10 of the leather after it has been gilded with a thin coating of gilt, silver, aluminum or their compounds when applied to the surface of the leather in sheet form.

Another object of my invention is to provide a leather coating or covering that will 15 not wash off when wet or moistened and will be durable for a long period of time.

A further object is to provide a leather with a bright, burnished, gilded surface that 20 will not be subject to cracking by reason of the flexing of the leather in the complete article of manufacture.

So far as I am aware, shoes, slippers and other articles of manufacture have heretofore 25 been gilded by the application of gold, silver or aluminum leaf by first applying a coating of gelatine or starchly preparation to the surface to cause the leaf to adhere. This preparation yields to moisture and to 30 a certain degree to extreme temperatures with the result that when the gilded surface is wet, the gilt easily rubs off. Furthermore, the gelatine hardens and becomes stiff when dry and cold, and the gilt plating cracks when the leather is flexed.

I have discovered that by the use of a proper sizing, such as "Japan size" that a much more durable coating may be made than with the use of gelatine or of starch 40 preparations, but it is very difficult to properly plate or coat with Japan size due to its quick drying properties. This is especially so in the case where the leather is dry and relatively stiff as the size is quickly absorbed by the leather and dries before the sheet of plating material is firmly attached and also for the reason that the thin flexible leather in bending cracks the gilt more or less.

These difficulties and others have been entirely overcome by the discovery that a thin coating of raw or boiled linseed oil or its equivalent, such as household oil varnish may be applied to the leather before 55 the Japan sizing is applied thereto which

will open the pores of the leather and when the size is applied, the oil acts on the size to slow up the drying action, thus allowing sufficient time to apply the leaf after the size has dried to a tacky condition. This 60 practice does not endanger the spoiling of the leaf or mussing the surface of the leather. After the size has dried to a strong tacky condition, the leaf is laid over the leather and by a smooth rubbing motion forced into intimate contact with the leather, the fingers pressing on the leaf in such a manner as to bring out the grain of the leather in relief and hold the plating in the interstices of the grain in a very satisfactory manner.

The action of the oil not only slows up the drying properties of the size but increases the flexibility of the surface of the leather so that the plating enters into more 75 intimate contact with the leather and in consequence the plating will not easily wear off when wet.

After the plating operation is completed, the surface may be burnished with proper 80 burnishing tools if desired or may be brushed with a fine wire brush to give a stippling effect, if this kind of a finish is desired.

Instead of coating the leather directly as 85 above set forth, I may add a few drops of the oil or varnish to an ounce of the Japan size, say four or five drops, to modify the action, or slow up its drying properties, and increase the flexibility of the leather. When 90 applied to the leather as a coating, the leaf may be applied as above set forth and very good results may be thus obtained by this practice.

It is obvious that I may use powdered 95 metal instead of the sheet form, as a covering for the leather, and I therefore do not wish to be limited to the use of sheet covering only but contemplate that my invention shall cover the use and application of a 100 slow drying oil in combination with the size of the character set forth for the purpose and use specified.

Having described my invention, what I now claim as new and desire to secure by 105 Letters Patent of the U. S. is:

1. The process of finishing leather which consists in applying to its surface a size of the character described in the presence of linseed oil to retard its drying properties 110

substantially free from pigment such as by a separate application therewith, and then covering said surface with a gilt.

2. The process of finishing leather which 5 consists in applying to its surface a size of the character described in the presence of a fast drying oil substantially free from pigment and then covering said surface with a gilt.

10 3. The process of finishing leather which consists in applying to its surface a size of the character described in the presence of a fast drying oil substantially free from pigment to retard its drying properties such as 15 by a separate application therewith, and then covering said surface with a sheet gilding.

4. The process of finishing leather which 20 consists in applying to its surface a fast drying oil substantially free from pigment and size mixture, covering said surface with sheet gilding and then rubbing the surface to bring out the grain of the leather.

5. The process of finishing leather which 25 consists in applying to its surface a size of

the character described in the presence of a fast drying oil substantially free from pigment, covering said surface with sheet gilding, rubbing the surface to bring out the grain of the leather and then burnishing the 30 coated surface.

6. The process of finishing leather which 35 consists in applying to its surface a size of the character described in the presence of a fast drying oil substantially free from pigment, covering said surface with sheet gilding and then stippling the coated surface.

7. The process of finishing leather which 40 consists in applying thereto a fast drying oil substantially free from pigment to increase its flexibility, covering said oiled surface with a size of the character described, applying sheet metal gilding to the surface, rubbing the gilded surface to force the metal into intimate contact with the pores of the 45 leather and then burnishing the gilded surface.

In testimony whereof I affix my signature.

FERDINAND WYCLIFFE ELLINGTON.